

Jan. 25, 1927.

1,615,392

J. S. LITTLE

# METHOD OF AND APPARATUS FOR MAKING FIBROUS ARTICLES

Filed March 26, 1923



Inventor  
John S. Little  
by H. C. Patterson.  
Atty.

## UNITED STATES PATENT OFFICE.

JOHN SHIRLEY LITTLE, OF LA GRANGE, ILLINOIS, ASSIGNOR TO WESTERN ELECTRIC COMPANY, INCORPORATED, OF NEW YORK, N. Y., A CORPORATION OF NEW YORK.

## METHOD OF AND APPARATUS FOR MAKING FIBROUS ARTICLES.

Application filed March 26, 1923. Serial No. 627,712.

This invention relates to methods of and apparatus for making fibrous articles, and more particularly to a method of and apparatus for coating cores.

- 5 An object of the invention is to produce a core having a coating of pulp thereon which is attached to the core solely by an intermingling of the fibers thereof and without the use of any adhesive substance.
- 10 Other objects of the invention are to produce a fibrous sheet consisting solely of intermingled pulp fibers and to color or otherwise treat the sheet in the process of its manufacture.
- 15 A further object of the invention is to treat pulpous material associated with a core for rendering the resultant core coating distinctive.
- Additional objects are to simultaneously 20 treat and to simultaneously apply distinctive indications to a plurality of portions of fibrous material simultaneously produced from a common supply of pulpous material.
- Briefly, the method consists in depositing 25 wet, pulpous material on a foraminous member giving a distinctive indication, such as by applying coloring material, to or otherwise treating the pulpous material in sheet form and then removing the moisture from 30 the sheet. In case a core is being coated the treated pulpous material is formed around the core to constitute a homogeneous coating therefor before the moisture is completely removed. When a plurality of sheets or 35 ribbons are being produced simultaneously, or a plurality of cores are being coated simultaneously, the sheets, ribbons or coatings are selectively or individually treated or colored.
- 40 When coated cores are employed in massed form as in the case of insulated electrical conductors formed into a cable it is often desirable to easily distinguish certain of conductors. This is frequently accomplished by 45 selectively coloring the coatings or insulation of the conductors to be identified.

When coated cores are woven to produce sheets it is also often desirable to employ differently colored coatings to produce patterns or some desired artistic effect.

Since it is of advantage to produce simultaneously differently colored sheets, ribbons or coated cores with the same machine or from a common supply of coating material, it is of advantage to color the coating ma-

terial after it is individually associated with the core.

In some cases it may be desirable to apply sizing to or to otherwise individually treat pulpous material placed on the cores while 60 the cores are being coated.

The drawings illustrate as an apparatus by which the method may be practiced, the apparatus being especially designed for coating cores in strand form, but it is to be 65 understood that other apparatus may be devised for coating cores in other forms without departing from the spirit and scope of the invention.

The word "pulp" as used in the specification and claims is to be understood as defining and including any cohering fibrous mass whether suspended in a liquid, moist, or substantially dry.

In the accompanying drawings—

Fig. 1 is a side elevation of a preferred apparatus by which the method may be practiced;

Fig. 2 is a fragmentary end view in section, of the cores and the structure for applying distinctive identifications to a plurality of cores.

Figs. 3, 4 and 5 are enlarged views showing the form of the pulp coating on each core as it is delivered from the foraminous member, the squeezing rolls, and the combined identifying and squeezing rolls respectively, while

Figs. 6 and 7 are enlarged views showing the form of the pulp coating on the core during the forming operation and after such operation is completed respectively.

The steps of the method will be readily understood from a detailed description of the apparatus by which the method may be 95 practiced.

Referring to the drawings in detail in which like reference numerals designate similar parts throughout the several views of the apparatus, the apparatus comprises a 100 drum 10 which is partially submerged in a liquid containing pulp within a trough 11. The drum 10 comprises a pair of metal sides and a peripheral portion 12 secured thereto. The portion 12 is provided at intervals with 105 a plurality of large perforations 13 arranged in rings, each ring being covered with a narrow strip of large wire mesh 56 over which a fine wire mesh 14 is placed as shown more clearly in Fig. 2. The drum has 110

- a centrally disposed tubular axle 15 which is rotatably mounted in suitable bearings 16 carried by the framework 17 which supports all of the elements of the apparatus.
- Pulpous material is strained onto the wire mesh strips 14 as the drum 10 is rotated in the tank by maintaining the level of the mixture within the drum 10 at a lower level than that of the pulp liquid in the tank 11, 10 as indicated by dotted lines A and B respectively. This difference in levels is maintained by a siphon pipe 18 which has its inlet opening submerged in the liquid within the drum and its discharge through the 15 tubular axle 15. A continuous circulation of pulp liquid is maintained in the tank 11 by feeding the pulp liquid from a supply tank (not shown) into the tank 11 by means of a pipe 19 and out of said tank through a 20 pipe 20 into a receiving tank (not shown), from which it is pumped back into the supply tank in any suitable manner. As the drum 10 rotates in the tank 11, due to the 25 difference in levels of the liquid in the drum and the tank, the liquid in the tank will pass through the strips of fine wire mesh 14 and the associated perforations 13 in the peripheral portion 12 of the drum 10, straining the pulp onto the outer surfaces of the strips.
- The cores to be coated, which are illustrated as being four in number, are fed from suitable supply spools 30 over idler rolls 31 into the pulp liquid in the tank 11 and into contact with the pulpous material which 35 has been deposited upon the foraminous strips 14.
- Attention is called to the fact that the idler rolls 31 are so spaced from the periphery 40 of the drum 10 that the cores are held out of contact with those sections of the foraminous strips 14 which are near the surface of the liquid in the tank, whereby pulp is strained onto such sections before the strands or cores are brought into contact therewith.
- The first deposit of pulp on the foraminous strips is indicated by the letter C, while as the drum revolves in the tank additional amounts of pulpous material will be deposited on the cores and upon the associated foraminous strips, forming a thicker coating indicated by the letter D. The drum 10 is rotated in the direction indicated by the arrow 45 and the pulp on the foraminous strips 14 thereof, together with the associated cores 50 are brought into contact with a felt covered roll 24. The periphery of this roll has a foraminous portion formed of fine wire mesh and when the pulp on the foraminous strips of the drum are brought into contact therewith, the "free liquid" so to speak in the pulp mixture will be squeezed out partially through the foraminous strips and partially through the felt and the associated 55 foraminous portion of the roll 24. The partially dried pulp adheres to the felt in the

form of ribbons, with the cores substantially centrally located therein, as shown in Fig. 3, and the cores with the pulp ribbons attached pass around the roll 24 and between it and a second felt covered roll 27. The 70 rolls 24 and 27 are carried by suitable brackets 21 supported by the framework 17 the roll 24 being positioned to engage the foraminous strips 14 of the drum 10 with a slight pressure. The rolls 24 and 27 are 75 forced together by any suitable tension means which is adjustable to exert the proper pressure between the cores and the pulp ribbons as they pass between the rolls, this pressure serving to mat the pulpous material and 80 secure it to the core to such an extent that as the cores leave the rolls they will carry the pulp ribbons with them. From the rolls 24 and 27 each of the cores with its pulp ribbon attached is passed between a pair of combined squeezing and treating rolls 29 and 30 which are also forced together by any suitable means adjustable to present the proper pressure on the cores and the pulp ribbons as they pass between the rolls, these 85 rolls also serving to remove some moisture from the pulp ribbon and to more firmly mat the fibers of the ribbon and attach it to the core.

Associated with the pairs of treating and squeezing rolls 29 and 30, which are mounted upon brackets 28 supported by the framework 20, are receptacles 44 to 47 inclusive supported by brackets 50 also attached to the framework 20. Extending from the bottom of each of the receptacles or tanks 44 to 47 inclusive is a suitable pipe including a hand operated valve and having a spray nozzle or other suitable means through which suitable coloring, sizing or other 105 chemical, which is to be applied to the coating, may be fed. The liquid flowing from each of these tanks is deposited upon the corresponding roll 29 and as such roll is brought into contact with the partially dried pulp 110 attached to the associated core, the liquid is absorbed by the pulpous material and flows throughout such material, the rolls 29 and 30 also assist in thoroughly distributing such liquid and to remove the surplus thereon. Thus in case a dye is used the entire ribbon is uniformly colored.

As it is evident from the drawing, the tanks 44 to 47 inclusive may contain different colors or different chemicals so that the various ribbons may receive different treatment, although the pulp from which they are formed is taken from a common supply. The construction of the pulp coating as it leaves the rolls 29 and 30 is shown in Fig. 5.

From the last mentioned rolls each core with its ribbon pulp is drawn through a former 34 which wraps the projecting edges of the ribbon around the core and around each other, the appearance of the coating

after it is first acted on by the former and after the forming action is completed being shown clearly in Figs. 6 and 7 respectively. The former causes a thorough intermingling 5 of the pulp fibers and shapes the coating so that it embraces the core and conforms to the shape thereof. This step of the process forms the coating into a mass so homogeneous that upon cutting the core and the coating, the latter will not fray or ravel and will not become easily detached from the core.

The former indicated by the reference numeral 34 is illustrated as being of the same type as that fully shown and described in a 15 co-pending application of H. G. Walker and A. T. March, Serial No. 547,923, filed March 29, 1922. Reference is made to such application for a full disclosure thereof. The former comprises essentially two plates, 41 20 and 42, which wrap the projecting edges of the pulp ribbon around each other and around the core in much the same manner as though the core and pulp ribbon were rolled on a table top with the palm of the 25 hand.

Each core with its formed coating is drawn from the associated former and subjected to a mechanism for thoroughly drying out the coating. The means shown for 30 performing this step of the process is a pair of wide hollow drums 51 and 52 heated internally and having a plurality of grooves (not shown) formed thereon, which receive the core, guides (not shown) being provided 35 for directing the core over first one drum and then the other until it has traversed all of the grooves on both drums, after which it is stored on a receiving drum 54. The drums 51 and 52 are revolvably mounted on suitable 40 bearings carried by vertical standards supported by the framework. The receiving drum 54 is also revolvably mounted on bearings supported by the framework, the drums being suitably driven by a suitable 45 belting system.

Although it has been stated that the primary object of the invention is to apply a coating of pulp to a core without the use of any adhesive substance, the process herein 50 disclosed may be used with a pulp mixture containing a sizing substance, or the pulp may be deposited on a core which has been previously treated with an adhesive agent without departing from the spirit and scope 55 of the present invention. It is evident that the dye or other agent may be deposited upon the ribbon in a dry state instead of liquid form, since it will be readily absorbed by the ribbon, due to the slightly moist condition of the ribbon when the agent is applied.

What is claimed is:

1. A method of coating a core with pulpous material which consists in associating a 65 core with pulpous material in such manner

that the material is held on the core solely by a felting of the pulp fibers, subjecting the pulpous material to a chemical to constitute a distinctive indication and then forming the material on the core to constitute a coating 70 having a curved outer surface.

2. A method of coating a core with pulp which consists in depositing pulpous material on a core in such manner that the material is held on the core solely by a felting 75 of the pulp fibers, coloring the deposited material and then forming the material on the core to constitute a coating conforming with the shape of the core.

3. A method of coating a core with pulp 80 which consists in associating a core with a sheet of pulpous material in such manner that the material is held on the core by a felting of the pulp fibers, coloring the material retained on the core and then wrapping 85 the said material around the core to constitute a coating therefor having a substantially circular outer surface.

4. A method of coating a core with pulp which consists in depositing pulpous material in the form of a ribbon longitudinally 90 of the core held on the core by a felting of the pulp fibers, subjecting the ribbon to a chemical to constitute a distinctive indication therefor, and then wrapping the ribbon 95 laterally around the core to constitute a coating therefor conforming with the shape of the core.

5. A method of coating a core in strand 100 form with pulp, which consists in depositing pulpous material on a foraminous member, bringing the core into contact with the deposited material, removing the core and the material from the foraminous member, applying an agent to the deposited material, 105 and then forming said deposited material on the core to constitute a coating therefor conforming with the shape of the core.

6. A method of coating a core in strand 110 form with pulp, which consists in subjecting a core to liquid containing pulp in such manner that pulp is applied to the core, applying a coloring agent to the deposited material, and forming said material on the core to constitute a coating therefor having a curved outer surface.

7. A method of coating a core in strand 115 form with pulp, which consists in applying wet pulpous material to a core in such manner that the material is held on the core by a felting of the pulp fibres, applying a coloring agent to said material, forming the deposited material on the core to constitute a coating therefor conforming with the shape of the core, and removing substantially 120 all the moisture from said coating.

8. A method of coating a core in strand 130 form with pulp, which consists in depositing pulpous material on a foraminous member, bringing the core into contact with the

deposited material, removing the core and the deposited material from the foraminous member, coloring the deposited material, and then forming the colored material on the 5 core to constitute a homogeneous coating therefor having a substantially circular outer surface.

9. A method of coating a core in strand form with pulp, which consists in depositing wet, pulpy material on a foraminous member, bringing the core into contact with the deposited material, removing the core and the deposited material from the foraminous member, removing some of the moisture from the deposited material, coloring the deposited material, and then forming the said material on the core to constitute a homogeneous coating therefor conforming with the shape of the core.

20 10. A method of coating a core in strand form with pulp, which comprises depositing pulpy material on a foraminous member, bringing the core into contact with the deposited material, removing the core and the 25 deposited material therefrom, depositing a coloring agent on another member, causing relative movement between the second mentioned member and the deposited material on the core to thereby color the material and 30 to remove moisture from the material, and then forming the colored material to constitute a homogeneous coating for the core conforming with the shape thereof.

11. A method of simultaneously coating a 35 plurality of cores in strand form with pulp, which comprises depositing pulpy material on a foraminous member, bringing a plurality of cores into contact therewith, removing the cores and the deposited material 40 therefrom, depositing coloring agents on a plurality of members, causing relative movement between the deposited material on each of the cores and one of the second mentioned members to color the material on each core 45 and to remove moisture therefrom, and then forming the material associated with each core to constitute a coating for the core conforming with the shape thereof.

12. A method of coating a plurality of 50 cores in strand form with pulp, which consists in depositing wet pulpy material upon the cores, applying coloring matter to the pulpy material on certain of the cores, and then forming the pulpy material on the 55 cores to constitute coatings thereon having a substantially circular outer surface.

13. In a machine for coating a core in strand form with pulp, a receptacle for containing a supply of fluid containing pulp, 60 a member, means for causing relative movement between said member and said fluid whereby pulp is deposited on said member, means for causing engagement between the core to be coated and the member whereby 65 pulpy material is deposited on said mem-

ber and said core, means for removing the core and the deposited material from the member and removing some of the moisture from the material, a receptacle for containing a supply of coloring matter, an outlet in 70 the receptacle, means for causing relative movement between the material and the outlet whereby coloring matter is deposited from the receptacle upon the material, and means individual to each of the cores for 75 forming the material thereon to form a homogeneous coating therefor.

14. In a machine for simultaneously coating a plurality of cores in strand form with pulp, a receptacle for containing a supply of 80 fluid containing pulp, a foraminous member, means for causing relative movement between said member and said fluid whereby pulp is deposited on said member, means for causing engagement between the cores and 85 the member whereby pulpy material is deposited on said cores, means for removing the cores and all of the deposited material from the member and removing some of the moisture from the material, each of said receptacles containing a plurality of receptacles, a supply of coloring matter, means for causing relative movement between the material on the cores and the receptacles, an outlet means for each receptacle for selectively applying coloring matter therefrom to the material associated with one of the cores, means for removing moisture from the portions of material, and mechanism individual to each of the cores for forming the 90 100 pulpy material applied thereto into a coating conforming with the shape of the core.

15. A method of coating a core in strand form, which consists in applying unfinished paper to the core in such manner that it is 105 held on the core by an intermingling of the fibres thereof, applying a coloring agent to the unfinished paper, and then completing the fabrication of the paper on the core to constitute a coating thereon conforming with 110 the shape of the core.

16. A method of coating a core in strand form, which consists in applying a ribbon of unfinished paper to the core, applying a 115 coloring material to said ribbon, and then completing the fabrication of the unfinished paper on the core to form a paper coating on the core conforming with the shape of the core.

17. A method of coating a core in strand form, which consists in applying a ribbon of unfinished paper to the core longitudinally thereof, applying a coloring material to said ribbon, and then wrapping the said ribbon laterally around the core and completing the fabrication thereof into a paper coating on the core.

In witness whereof, I hereunto subscribe my name this 9th day of March A. D., 1923.

JOHN SHIRLEY LITTLE.